

## UNITED STATES PATENT OFFICE.

ROBERT BIGHAM SMITH, OF MACON, GEORGIA, ASSIGNEE, BY DIRECT AND MESNE ASSIGNMENTS, TO BORNE, SCRYSER COMPANY, OF NEW YORK, N. Y., A CORPORATION OF NEW JERSEY.

## METHOD OF OILING COTTON RAW STOCK.

No Drawing.

Application filed November 8, 1924. Serial No. 748,765.

*To all whom it may concern:*

Be it known that I, ROBERT BIGHAM SMITH, a citizen of the United States, and resident of Macon, in the county of Bibb and State of Georgia, have invented certain new and useful Improvements in Methods of Oiling Cotton Raw Stock, of which the following is a specification.

The invention relates to a method of conditioning by oiling cotton fibre when in the form of raw stock and before it has been carded and spun into yarn.

In the manufacture of cotton into yarn the fibres are carded, paralleled, and twisted around each other. Cotton fibre is distinguished from all other fibre in the peculiar twist it possesses and by its long, soft, flexible, and silky staple. While its peculiar soft texture renders cotton fibre comparatively easy to manipulate and work through the different machines incidental to its manufacture into the finished product, still the machining of these soft, silky fibres gives rise to certain difficulties in the machining of the stock. For instance, the drawing and spinning operation generates static electricity on the cotton fibre which causes the fibres to resist each other, to stand apart, and flare out at right angles to the length of the yarn. This tendency towards surface disintegration not only weakens the resulting yarn, but seriously interferes with the proper processing of the fibre.

Attempts have been made to dissipate the static charges on the sliver by mill humidification, which consists in moistening the air, but this has not proven satisfactory. Water has been sprayed upon the fibre to neutralize the formation of this static electricity, but the water evaporated and otherwise this treatment has not proven effective. The cotton stock has been sprayed with solutions of soap and water, or emulsions of soaps and vegetable oils in water. The objection to the use of the soap and water treatment is that the soap disintegrates with age, changing its chemical nature and physical form, thereby defeating its purpose as a lubricant and softener. The use of vegetable oils and emulsions or mixtures of these oils is objected to for the same reason as the soaps, that is, these oils are drying or semi-drying

in nature or are readily oxidizable and break down, dry up and form compounds which are sticky and otherwise objectionable for the purpose of treating cotton to assist in the manufacture of the fibre into goods for the market. The use of these solutions and liquids has been confined to the manufacture of waste cotton and cotton of short fibre length primarily to prevent the excessive losses in manufacture and hold as much weight to the finished product as possible and without intent to affect any conditioning of the material.

The primary object of the invention is to treat the raw cotton stock either while in bulk or during one of the initial machining operations in such way as will minimize the formation of static electricity and incidentally insure the retention and utilize in the resulting sliver all of the long, fine fibres present in the stock.

Broadly, this object is attained by subjecting the raw cotton stock to a preliminary oil treatment with the oil in a finely divided liquid form and in relatively small amounts.

Causing a small quantity of a suitable oil to permeate the stock results in the fine fibres adhering substantially in parallelism during the drawing operation and provides internal lubrication which reduces frictional resistance between the material and the machine parts during the succeeding machining operations, as well as reduces the resistance between the individual fibres, as they adjust themselves to their determined location in the body of the yarn as it is formed by these machining operations.

Due to its inherent chemical properties and efficient lubricating properties a pure mineral lubricating oil has been found best for the purpose. This oil may be used in its natural color after a suitable refining has been carried out to render it of the proper viscosity and gravity for the purpose intended.

While the use of mineral or petroleum oil, used pure and without other ingredients, is featured in this disclosure due to its cheapness and efficiency in its softening and lubricating quality other less efficient oils may be used for example castor oil and lard oil.

In some instances where it is of advantage to ship the finished yarn in its natural or grey state and while impregnated with a small quantity of oil, the oil used should be 5 such as will not color the product. In such cases it is herein intended that a colorless, bleached or waterwhite lubricating mineral oil be used the commercial grades of which are not regarded as volatile and can have a 10 flash point as low as 110° F.

The oil is sprayed or sprinkled onto the raw stock before assuming the drawn out stage of yarn and as the fibres are pulled over one another and repeatedly doubled in 15 incidental to the succeeding machining operations, the oil will be evenly distributed and absorbed so that practically every fibre will have approximately its proportionate share of oil.

20 The amount of oil used will depend on the viscosity and gravity of the oil, upon the character of the cotton fibre and upon the use to which the resulting yarn is to be placed. In general, sufficient oil must be 25 used to attain the desired results, but not so much as will interfere with the passage of the material through the machinery. In the case of mineral oil, which has been found most practical for the purpose, the amount 30 used varied from one-half to one to four percent by weight of the stock treated. It has been found that if the weight of the oil used materially exceeded four percent of the weight of the material treated, it will 35 cause the stock to adhere to the machine parts and prevent the proper processing of this stock into finished goods.

When it is desired to remove the oil from the finished material certain emulsifying 40 agents, well known to those skilled in the art, may be used; the general procedure is to add to the boiling out process of the goods suitable soaps, borax, alkali or other chemicals which substances will remove 45 from the goods the mineral oil when applied in the manner described in this process.

The presence of this small quantity of mineral oil does not interfere with the 50 chemical or any subsequent treatment of the stock for manufacturing purposes when applied in the manner described in this process. Its presence is an advantage in certain operations such as in a knitting or weaving 55 where it insures lubrication and an easy sliding of the knitting yarn through the various parts of these machines and renders unnecessary any separate oiling of the yarn. The yarn made from stock treated as herein described produces goods of a softer and more 60 supple nature than would be the case if this pre-oiling treatment were omitted.

It has been found experimentally that as 65 the result of the treatment herein disclosed the pitch angle of the spirals forming the cotton fibre becomes more sharply inclined

thus causing the length of the fibres to become longer. It has also been found that the breaking strength of the yarn is increased.

Having thus described my invention, I 70 claim:

1. In the art of preventing the presence of static electrical charges from affecting the fibres during the drawing process incidental to the manufacture of yarn from raw 75 cotton stock, the method which includes the step of subjecting the stock to a treatment of a non-volatile oil in a finely divided liquid state before the stock is drawn.

2. In the art of treating raw cotton stock, 80 the method which includes the step of applying lubricating oil in liquid form to the stock prior to the completion of the drawing operation and permitting the oil to permeate the stock during the drawing of the 85 fibres.

3. In the art of treating cotton raw stock incidental to the manufacture of the same into cotton yarn having a soft, supple character, the method which consists in spraying 90 the stock with a non-volatile mineral oil prior to the completion of the drawing process.

4. In the art of treating raw cotton stock, 95 the method which includes the step of treating the stock with a non-volatile mineral oil, and with the oil present in an amount substantially less than four percent by weight of the stock treated.

5. In the art of treating raw cotton stock, 100 the method which consists in spraying a colorless lubricating mineral oil on to the stock and manipulating the stock to insure the permeation of the oil through the same.

6. In the art of treating cotton fibres, during the process of drawing the fibres into 105 yarn, the method which consists in causing a colorless lubricating oil to permeate the fibres.

7. In the art of treating cotton fibres, during the process of drawing the fibres into 110 yarn, the method which consists in causing an oil to permeate the fibres, said oil being present in liquid form and in an amount less than four percent by weight of the 115 amount of fibre present.

8. In the art of treating cotton fibres for the purpose of preventing the undesirable effects of the presence of static electricity thereon, the method which consists in diffusing through the material a charge of lubricating oil in liquid form. 120

9. In the art of treating cotton fibres for the purpose of preventing the undesirable effects of the presence of static electricity thereon, the method which consists in diffusing through the material a charge of mineral oil while in a finely divided liquid state and in an amount less than four percent by weight of the material treated. 125 130

10. In the art of treating cotton fibres, the method which includes the step of causing lubricating mineral oil to permeate the fibres and thus provide for internal lubrication.

11. An untwisted cotton containing a lubricating oil present in an amount of less than four per cent by weight of the cotton and on which the oil is distributed uniformly throughout the same.

12. A soft supple cotton saturated with a lubricating mineral oil present in an amount not less than one-half of one percent by

weight or not more than four percent by weight of the cotton.

15

13. A cotton product comprising untwisted and undrawn fibres treated with liquid oil to cause the pitch angle of its spiral fibres to become more sharply inclined and thus cause the length of the fibres to become longer than the same fibres when not so treated.

20

Signed at Macon, in the county of Bibb and State of Georgia, October A. D. 1924.

ROBERT BIGHAM SMITH.